# EUROPEAN PATENT SPECIFICATION

(11) **EP 0 105 731 B1**
(45) Date of publication and mention of the grant of the patent: **09.08.1989**
(21) Application number: 83305893.6
(22) Date of filing: 29.09.1983
(51) Int. Cl.: D04H 1/54

(54) **Double belt bonding of fibrous web comprising thermoplastic fibers on steam cans**
Verfestigung einer thermoplastische Fasern enthaltenden Faserbahn zwischen zwei Bändern, auf dampfbeheiztem Zylinder
Consolidation d'une nappe de fibres contenant des fibres thermoplastiques entre deux courroies, sur des cylindres chauffés à la vapeur

(30) Priority: 30.09.1982 US 430308
(43) Date of publication of application: 18.04.1984
(73) Proprietor: CHICOPEE, New Brunswick New Jersey 08903 (US)
(72) Inventor: Mays, Alfred T., East Windsor New Jersey 08520 (US); Wereson, Nicholas, Spotswood New Jersey 08884 (US)
(74) Representative: Jones, Alan John

(56) References cited:
- FR-A- 1 059 617

## Description

### BACKGROUND OF THE INVENTION

Method and apparatus for drying and heat setting fibrous webs about steam cans are known. The method involves utilizing a carrier belt to carry the web in a serpentine pattern about a series of steam cans. The method and apparatus may also utilize cooling cans about which the web is subsequently carried. The prior art encompasses many variations in the above method and apparatus. U.S. Pat. No. 1,519,239 to Clay discloses a molding apparatus for fibrous sheet material. The fibrous sheet is passed around and between a series of pressure rollers. The initial pressure roller nip is heated and subsequent pressure roller nips may be cooled. Endless carrier belts are provided to move the fibrous sheet material through and around the pressure rollers.

U.S. Pat. No. 3,671,365 to Cover Jr., et al., discloses an apparatus for compressing and cooling a fibrous web. The fibrous web is fed between an upper series and a lower series of rollers comprising the compression frame. A carrier belt is mounted about each of the upper and lower series of rollers. U.S. Pat. No. 3,442,740 to David, discloses a process and apparatus which comprises a modification of the palmer dryer and method used to dry and heat fibrous webs. The palmer dryer comprises a heated roll and a flexible endless belt which travels around the roll. A web is fed between the belt and the roll, and travels about the roll while under the belt. In the modification described in the David patent, the web is doffed from the heating roll and travels around another cooling roll or drum. In the method of the present invention, the fibrous web is maintained between two belts as the belts travel about spaced heated cans and optionally thereafter spaced cooling cans.

FR-A-1059617 describes a process for making paper-like materials from thermoplastic fibres. In the process, a web of fibres laminated between carrier belts is conducted around heating rolls such that the web is heated first from one side, then the other. When passing over the heating rolls, pressure is applied on the two belt laminate by pressure rolls. The belts are such that pressure is distributed over the web in punctiform manner.

### SUMMARY OF THE INVENTION

The present invention comprises a method and apparatus for producing a fabric from a fibrous web comprising at least 5 percent thermoplastic fibers. As used herein, the term 'thermoplastic fibres' encompasses such conjugate fibers. The method comprises
(a) superimposing a fibrous web comprising at least 5 percent thermoplastic fibers on a first endless carrier belt;
(b) superimposing a second carrier belt on said web so as to form a two belt laminate with said web sandwiched between the first and second endless carrier belts;
(c) causing said two belt laminate to travel in a path consecutively around first and second heated rolls, which are offset from each other and spaced apart a sufficient distance to avoid a compression nip between said first and second heated rolls, the peripheral surfaces of said first and second heated rolls cooperating to provide a portion of said path whereon said two belt laminate travels out of contact with said first and second heated rolls, so as to initially apply heat to a first side of said web as said two belt laminate is directed around said first heated roll and thereby fuse the thermoplastic fibers to fibers adjacent the first side thereof and to thereafter apply heat to a second side of said web as said two belt laminate is directed around said second heated roll and thereby fuse the thermoplastic fibers to fibers adjacent the second side thereof; and
(d) cooling the two belt laminate after it has travelled around the first and second heated rolls so as to cool the fibers in the web sandwiched between the first and second endless carrier belts.

Low shrink thermoplastic fibers may be used, or alternatively, tension may be applied to the web through the belts to prevent substantial shrinkage of the web. Optionally, the fibers may be cooled by passing the web and two belts about spaced cooling cans. The thermoplastic fibrous material formed by the apparatus and method of the present invention have excellent cross directional strength.

### BRIEF DESCRIPTION OF THE DRAWINGS

The Figure is a schematic side view of the method according to the present invention.

### DESCRIPTION OF THE DRAWINGS

The present invention utilizes a series of spaced heated rolls, such as the steam cans currently used to bond and heat set fibrous webs, in a new and unique process for producing a fabric containing thermoplastic fibers. The heated rolls or steam cans depicted at 1 in Figure 1 are rotatably mounted to a frame (not shown). The rolls or cans are spaced from each other, and in no way provide a compression nip. A first endless carrier belt 3, is wound about means 5, for causing said first belt to travel in a serpentine path about the rolls. A second endless carrier belt 7, is wound about means 9, for causing the second belt to travel along an initial path 11, spaced from said first belt, and then _{"}along said serpentine path about the rolls. Means 5' may be adjusted to impart different degrees of tension to the belts, lower tension yielding higher bulk fabrics and higher tension giving rise to less shrinkage. First and second carrier belts may be formed of, for example, polyester, stainless steel, teflon coated fiberglass, teflon, or bronze. The belts may vary in construction from, e.g., a 40 x 40 mesh to a substantially non-porous configuration. The belts preferably have good release properties, e.g., the teflon and teflon coated fiberglass belts. Another useful property in the belt is good heat transmission as exhibited by belts of bronze and stainless steel.

According to the method of the present invention, a web 13 comprising, e.g., low shrink thermoplastic fibers may be superimposed on said first carrier belt and the second carrier belt is superimposed on said web forming a two belt laminate 15 just prior to or as the belts begin to travel about the rolls. The rolls, which may be heated by any suitable means, melt and fuse the thermoplastic fibers to fibers in the web. The fibrous web is maintained between the two belts as it is removed from the last in the series of rolls and is maintained between the belts until the web cools. To facilitate cooling of the web, the belts may be passed around at least one cooling roll as shown in Figure 1 at 17. The cooling rolls are also spaced and in no way comprise a compression nip.

The present method and apparatus may utilize existing steam cans as the heated rolls used to fuse the low shrink thermoplastic fibers to form a fibrous material. By maintaining the web between the belts until the web is cooled, the method avoids the loss in cross directional strength due to drafting as a web is removed from a roll on one carrier belt. Also the use of two belts prevents sticking of the heated thermoplastic fibers of the web to the rolls and permits rapid handling of the web while heated, including immediately passing the web about cooling rolls. Low shrink thermoplastic monofils such as Eastman 4BC crystalline copolyester fibers may be used in the present invention, however, sheath/core polyethylene/ polyester conjugate fibers are preferred. The conjugate fibers may be eccentric, symmetrical sheath/core or side by side by side. Polyethylene/ polypropylene conjugate fibers may also be used. In all cases, means 5' may be used to adjust the tension and reduce shrinkage.

The foregoing description and drawing are illustrative but are not to be taken as limiting. Other variations and modifications are possible without departing from the scope of the present invention.

## Claims

1. Method of producing a fused nonwoven fabric comprising thermoplastic fibers, said method comprising:
(a) superimposing a fibrous web comprising at least 5 percent thermoplastic fibers on a first endless carrier belt;
(b) superimposing a second carrier belt on said web so as to form a two belt laminate with said web sandwiched between the first and second endless carrier belts;
(c) causing said two belt laminate to travel in a path consecutively around first and second heated rolls, which are offset from each other and spaced apart a sufficient distance to avoid a compression nip between said first and second heated rolls, the peripheral surfaces of said first and second heated rolls cooperating to provide a portion of said path whereon said two belt laminate travels out of contact with said first and second heated rolls, so as to initially apply heat to a first side of said web as said two belt laminate is directed around said first heated roll and thereby fuse the thermoplastic fibers to fibers adjacent the first side thereof and to thereafter apply heat to a second side of said web as said two belt laminate is directed around said second heated roll and thereby fuse the thermoplastic fibers to fibers adjacent the second side thereof; and
(d) cooling the two belt laminate after it has travelled around the first and second heated rolls so as to cool the fibers in the web sandwiched between the first and second endless carrier belts.

2. A method as in Claim 1, wherein the thermoplastic fibres are conjugate fibres.

3. A method as in Claim 2, wherein the conjugate fibres, are sheath/core polyethylene/polyes- ter fibres.

4. Apparatus for forming a fused nonwoven fabric comprising thermoplastic fibers, said apparatus comprising:
(a) a frame;
(b) first and second heated rolls rotatably mounted to said frame in offset relationship to each other, said rolls being spaced apart a sufficient distance to avoid a compression nip between said first and second rolls;
(c) a first endless carrier belt means mounted to said frame for travel in a path consecutively around said first and second heated rolls;
(d) a second endless carrier belt means mounted to said frame for travel along said path around said first and second heated rolls adjacent to said first belt means;
(e) means for superimposing a fibrous web onto said first belt means so that said first and second belts form a two belt laminate with said web sandwiched therebetween, said path being such that in use said two belt laminate is caused to travel in said path consecutively around said first heated roll to initially apply heat to a first side of said web and then around said second heated roll to apply heat to a second side of said web;
(f) the peripheral surfaces of said first and second heated rolls cooperating to provide a portion of said path whereon said two belt laminate travels out of contact with said first and second heated rolls; and
.(g) cooling means for cooling said two belt laminate after it has travelled around said first and second heated rolls to cool the fibers in the web sandwiched between first and second endless carrier belts.

5. An apparatus as in Claim 4 wherein said means for cooling comprises at least one cooled roll.

## Patentansprüche

1. Verfahren zur Herstellung eines verschmolzenen nicht gewebten Stoffes aus thermoplastischen Fasern, bestehend aus:
(a) Aufbringen einer Faserbahn, die zumindest 5% thermoplastische Fasern enthält, auf ein erstes endloses Förderband;
(b) Aufbringen eines zweiten Förderbandes auf die genannte Bahn zur Bildung eines aus zwei Bändern bestehenden Laminates mit der genannten Bahn in Sandwich-Anordnung zwischen den ersten und zweiten endlosen Förderbändern;
(c) der Bewegung des aus den beiden Bändern bestehenden Laminates auf einer Bahn aufeinanderfolgend um erste und zweite erhitzte Walzen, die gegeneinander versetzt und in einem genügenden Abstand voneinander angeordnet sind, um einen Preßspalt zwischen den genannten ersten und zweiten erhitzten Walzen zu vermeiden, wobei die Umfangsflächen der genannten ersten und zweiten erhitzten Walzen zusammenwirken, um einen Teil der Bewegungsbahn vorzusehen, auf dem das aus den beiden Bändern bestehende Laminat die Berührung mit den ersten und zweiten erhitzten Walzen verliert, um anfänglich Hitze auf eine erste Seite der genannten Bahn aufzubringen, wenn das aus den beiden Bändern bestehende Laminat um die genannte erste erhitzte Walze herumgeführt wird und dadurch die thermoplastischen Fasern mit Fasern zu verschmelzen, die der ersten Seite derselben benachbart sind, und um danach Hitze auf eine zweite Seite der genannten Bahn aufzubringen, wenn das aus den beiden Bändern bestehende Laminat um die genannte zweite erhitzte Walze herumgeführt wird und dadurch die thermoplastischen Fasern mit Fasern verschmolzen werden, die der zweiten Seite derselben benachbart sind, und
(d) Abkühlen des aus den beiden Bändern bestehenden Laminats nachdem es um die ersten und zweiten erhitzten Walzen herum bewegt worden ist, um die Fasern in der zwischen den ersten und zweiten endlosen Förderbändern sandwichartig angeordneten Bahn abzukühlen.

2. Verfahren nach Anspruch 1, bei dem die thermoplastischen Fasern konjugierte Fasern sind.

3. Verfahren nach Anspruch 2, bei dem die konjugierten Fasern eine Hülle aus Polyethylen und einen Kern aus Polyester aufweisen.

4. Vorrichtung zur Herstellung eines verschmolzenen nicht gewebten Stoffes aus thermoplastischen Fasern, bestehend aus:
(a) einem Gestell;
(b) ersten und zweiten erhitzten Walzen, die in dem genannten Gestell in versetzter Anordnung zueinander drehbar angeordnet sind, wobei die Walzen in einem genügenden Abstand voneinander angeordnet sind, um einen Preßspaltzwischen den ersten und zweiten Walzen zu vermeiden;
(c) einem ersten endlosen Transportband, das auf dem genannten Gestell auf einer Bewegungsbahn aufeinanderfolgend um die genannten ersten und zweiten erhitzten Walzen bewegbar ist;
(d) einem zweiten endlosen Transportband, das auf dem Gestell zur Bewegung längs der genannten Bewegungsbahn rund um die ersten und zweiten erhitzten Walzen in der Nähe des genannten ersten Bandes angeordnet ist;
(e) Mitteln zum Übereinanderanordnen einer Faserbahn auf dem ersten Band, so daß die ersten und zweiten Bänder ein aus zwei Bändern bestehendes Laminat bilden, wobei die genannte Bahn sandwichartig zwischen ihnen angeordnet ist, und daß die genannte Bewegungsbahn so beschaffen ist, daß beim Betrieb das genannte, aus den beiden Bändern bestehende Laminat veranlaßt wird, sich auf der genannten Bewegungsbahn aufeinanderfolgend um die erste erhitzte Walze zum anfänglichen Aufbringen von Hitze auf eine erste seite der genannten Bahn und dann um die genannte zweite erhitzte Walze zum Aufbringen vom Hitze auf eine zweite Seite der genannten Bahn zu bewegen; wobei
(f) die Umfangsflächen der genannten ersten und zweiten erhitzten Walzen zusammenwirken, um einen Teil der Bewegungsbahn vorzusehen, auf dem das Laminat aus den genannten beiden Bändern sich von den genannten ersten und zweiten erhitzten Walzen löst; und
(g) KÜhlmitteln zum Kühlen des aus den beiden Bändern bestehenden Laminates, nachdem es um die genannten ersten und zweiten erhitzten Walzen zur Kühlung der Fasern in der Bahn bewegt worden ist, die sandwichartig zwischen den ersten und zweiten endlosen Transportbändern angeordnet ist.

5. Vorrichtung nach Anspruch 4, wobei die genannten Mittel zum Kühlen aus mindestens einer gekühlten Walze bestehen.

## Revendications

1. Procédé de production d'un textile non tissé soudé comprenant des fibres thermoplastiques, qui comporte:
(a) la superposition d'une nappe comprenant au moins 5% de fibres thermoplastiques sur une première courroie porteuse sans fin;
(b) la superposition d'une seconde courroie porteuse sur ladite nappe pour former un lamifié de deux courroies, avec ladite nappe prise en sandwich entre la première et la deuxième courroies porteuses sans fin;
(c) la mise en circulation du lamifié des deux courroies sur un trajet conduisant successivement autour d'un premier et d'un second cylindres chauffés, qui sont désaxés l'un par rapport à l'autre et écartés d'une distance suffisante pour éviter un pincement par compression entre lesdits premier et second cylindres, les surfaces périphériques desdits premier et second cylindres chauffés coopérant pour délimiter une portion dudit trajet où passe le lamifié des deux courroies, sans contact avec lesdits premier et second cylindres chauffés de façon à apporter de la chaleur, au début à une première face de ladite nappe, quand ledit lamifié de deux courroies passe autour du premier cylindre chauffé et de façon à souder ainsi les fibres thermoplastiques aux fibres adjacentes de cette face, puis de façon à apporter de la chaleur à la deuxième face de ladite nappe, quand ledit lamifié de deux courroies passe autour du deuxième cylindre chauffé et de façon à souder ainsi les fibres thermoplastiques aux fibres adjacentes de sa deuxième face; et
(d) le refroidissement du lamifié des deux courroies après son passage autour du premier et du deuxième cylindres chauffés, de manière à refroidir les fibres de la nappe prise en sandwich entre la première et la deuxième courroie porteuse sans fin.

2. Procédé selon la revendication 1, dans lequel les fibres thermoplastiques sont des fibres complexes.

3. Procédé selon la revendication 2, dans lequel les fibres complexes sont des fibres gaine/coeur en polyéthylène/polyester.

4. Appareil de production d'un textile non tissé soudé comprenant des fibres thermoplastiques, cet appareil comportant:
(a) un châssis;
(b) un premier et second cylindres montés sur le cadre de manière à pouvoir tourner, désaxés l'un par rapport à l'autre, lesdits cylindres étant suffisamment écartés pour éviter un pincement de compression entre lesdits premier et second cylindres;
(c) une première courroie porteuse sans fin, montée sur ledit châssis, pour circuler sur un trajet passant consécutivement autour desdits premier et second cylindres chauffés;
(d) une seconde courroie porteuse sans fin, montée sur ledit châssis pour circuler le long dudit trajet autour desdits premier et second cylindres chauffés, de manière adjacente à ladite première courroie;
(e) des moyens pour superposer une nappe de fibres sur ladite première courroie de sorte que lesdites première et seconde courroies forment un lamifié avec la nappe prise en sandwich entre elles, ledit chemin étant tel que pendant le fonctionnement, le lamifié constitué de deux courroies circule sur ledit trajet, successivement autour dudit premier cylindre chauffé pour chauffer d'abord une première face de la nappe et ensuite autour dudit second cylindre chauffé pour chauffer la seconde face de ladite nappe;
(f) les surfaces périphériques desdits premier et second cylindres chauffés coopèrent pour délimiter une portion dudit trajet dans lequel le lamifié constitué de deux courroies circule sans contact avec lesdits premier et second cylindres chauffés; et
(g) des moyens de refroidir ledit lamifié constitué des deux courroies, après qu'il soit passé autour desdits premier et second cylindres chauffés pour refroidir les fibres de la nappe prise en sandwich entre la première et la deuxième courroies porteuses sans fin.

5. Appareil selon la revendication 4, dans lequel lesdits moyens de refroidissement comprennent au moins un cylindre refroidi.
